

## UNITED STATES PATENT OFFICE

1,957,354

PROCESS OF PROTECTING LIGHT METALS  
AGAINST CORROSION

Pierre Prier, Paris, France

No Drawing. Application April 26, 1932, Serial  
No. 607,670. In France April 27, 1931

3 Claims. (Cl. 148—6)

It is known to protect light metals and alloys either by formation of a layer of oxide by means of an electric current in the midst of a conducting solution, or by deposition of metallic oxides, with or without current, in the midst of an alkali and salt solution.

The present invention has for its object a process allowing to form a protecting layer, very resistant to corrosion, on aluminium, magnesium and their alloys.

An extremely satisfactory protection is obtained according to the present process by causing to react, on parts formed of light metals or alloys, an aqueous solution of one or more complex neutral soluble salts, the anion of which compulsorily comprises the fluorine element combined with one or more other elements, the cation being of any nature, but one of the constituent elements of the salt being placed above aluminium in the series of electro-chemical potentials.

The addition of bodies adapted to dissolve or precipitate the secondary bodies formed by the reaction (such as tartrates, citrates, fluorides, etc.,) can be effected without modifying the protection provided by the present process. These additions are not indispensable and do not constitute the essential feature of the present invention.

The rapidity and efficiency of the reaction increase with the temperature and reach their maximum at boiling point.

The duration of treatment of the metal with the bath is substantially of 15 to 20 minutes. It can be prolonged until the end of the reaction.

The following examples are given by way of indication and not in a limiting sense.

## Example I

|    |                                         |       |           |
|----|-----------------------------------------|-------|-----------|
| 40 | Fluovanadate of potassium               | ----- | 10 grs.   |
|    | Fluosilicate of sodium                  | ----- | 1 gr.     |
|    | Double tartrate of sodium and potassium | ----- | 1 gr.     |
|    | Water                                   | ----- | 1.000 cc. |

|    |                                           |       |         |
|----|-------------------------------------------|-------|---------|
| 45 | Example II                                |       |         |
|    | Double fluoride of potassium and titanium | ----- | 2 grs.  |
|    | Chromium fluoride                         | ----- | 1 gr.   |
| 50 | Fluoride of sodium                        | ----- | 0.5 gr. |

Water  
-----  
1.000 cc.

It has been found that the quantity of each of the constituents can vary within wide limits, but the best results have been obtained by means

of a solution composed according to the second above example.

It has also been found that the bath can be continuously used by eliminating the totality or a portion of the chemical compounds which are formed during the reaction by simple reagents containing in the anion the fluorine element and capable or not of generating the complex salts such as they are above defined.

By way of indication, the continuous action of the bath of the second above example can be ensured by addition of titanium fluoride.

Protecting coatings obtained in such baths have a high resistance to the usual oxidation agents and in particular to the saline mist and to the saline solution of perhydrol.

The parts treated according to this process are preferably subsequently coated with another protecting layer which can be composed of greases, oils, waxes, gums, tar, etc.

The present process is not limited to the above mentioned conditions and the quality and aspect of the protecting layer can be varied by modifying the concentration of the bath, or the temperature or duration of treatment, etc.

I claim:

1. Process for the formation of coatings for preventing the oxidation on articles made of light metals or alloys such as aluminium, magnesium, which consists in immersing the said articles in a solution comprising about 2 parts of double fluoride of potassium and titanium, 1 part of chromium fluoride and  $\frac{1}{2}$  part of fluoride of sodium for 1000 parts of water.

2. Process for the formation of coatings for preventing the oxidation on articles made of light metals or alloys such as aluminium, magnesium, which consists in immersing the said articles in a solution comprising about 2 parts of double fluoride of potassium and titanium, 1 part of chromium fluoride and  $\frac{1}{2}$  part of fluoride of sodium for 1000 parts of water, and in gradually adding fluoride of titanium to the said solution in the course of its use.

PIERRE PRIER. 100

105

110